

G. A. GUESS.  
PROCESS OF ELECTROLYTICALLY SEPARATING NICKEL FROM COPPER.  
APPLICATION FILED AUG. 14, 1917.

1,251,511.

Patented Jan. 1, 1918.



INVENTOR.

G. A. Guess.

BY J. Edward McCabe

ATTY.

# UNITED STATES PATENT OFFICE.

GEORGE A. GUESS, OF OAKVILLE, ONTARIO, CANADA.

## PROCESS OF ELECTROLYTICALLY SEPARATING NICKEL FROM COPPER.

1,251,511.

Specification of Letters Patent.

Patented Jan. 1, 1918.

Application filed August 14, 1917. Serial No. 186,147.

*To all whom it may concern:*

Be it known that I, GEORGE A. GUESS, of the town of Oakville, in the county of Halton, Province of Ontario, Canada, have invented certain new and useful Improvements in Processes of Electrolytically Separating Nickel from Copper, of which the following is a specification.

In the electrolytic recovery of nickel and copper from copper-nickel ores, the use of anodes of copper-nickel in an electrolyte of nickel sulfate and the plating out of the nickel on a nickel cathode is a process well known in the art of metallurgy, but in carrying out such a process many refinements have to be introduced to prevent the copper being re-deposited with the nickel. These special features introduce complications and expense which it is the object of my invention to avoid.

I attain my object by means which may be briefly described as follows. A substantially insoluble reagent is employed which will react with copper sulfate to form an insoluble copper compound and, preferably, an insoluble sulfate or a sulfate the presence of which in the electrolyte is not prejudicial. The insoluble re-agent is used to form in effect a screen or filter between the anode and cathode to intercept and precipitate the copper and thus prevent it depositing on the cathode. Suitable porous screening means are provided to prevent the re-agent contacting with the cathode.

The process is carried out in detail substantially as hereinafter more particularly described and by means of apparatus constructed in principle along the lines illustrated in the accompanying drawings in which—

Figure 1 is a diagrammatical vertical section of one form of the apparatus; and

Fig. 2 a similar view of a modification.

In the drawings like numerals of reference indicate corresponding parts in the different figures.

Referring particularly to Fig. 1, 1 is the electrolytic cell, 2 the anode, 3 the cathode and 4 the electrolyte. In the electrolyte I suspend pulverized calcium carbonate, which is maintained in suspension by any suitable means of agitation. The electrolyte also is preferably heated to a temperature of between sixty to eighty degrees centigrade. The cathode is shielded from contact with

the calcium carbonate by means of a porous cell 5.

In the form of apparatus shown in Fig. 2, the calcium carbonate may be in larger pieces and is maintained in contact with the anode by being placed in a porous cell of any suitable material surrounding the anode.

In each form, while the re-agent employed is present in the electrolyte, it is in contact only with the anode and the cathode is screened from contact with such re-agent. When electrolysis is carried on in apparatus such as described, the anode being of copper-nickel, the copper dissolved from the anode is precipitated in insoluble form as carbonate or hydroxid, and nickel only is plated on the cathode. The calcium of the calcium carbonate is precipitated as insoluble calcium sulfate.

It is essential to the carrying out of my process to employ a re-agent which will precipitate the copper in an insoluble form and which will result in the formation of a sulfate whose presence in the electrolyte in either solid form or in solution is not detrimental to the process.

Bearing this in mind it will be readily understood that carbonates of the other alkaline earths would satisfactorily serve my purposes; so also lime will be found to be an equivalent for the calcium carbonate, or limestone, which is the most satisfactory re-agent I have employed owing to its cheapness and the insoluble character of the sulfate formed. Nickel carbonate might also be employed as a substitute for the calcium carbonate. In this case, the nickel sulfate formed during the re-action enters into the electrolyte and becomes electrolyzed during the process.

What I claim as my invention is:—

1. A process of electrolyzing a nickel sulfate solution with the use of a copper-nickel anode which consists in employing in the electrolyte a substantially insoluble re-agent capable of forming with copper an insoluble compound and a sulfate whose presence in the electrolyte is not detrimental, while screening the cathode from contact with such re-agent.

2. A process of electrolyzing a nickel sulfate solution with the use of a copper-nickel anode which consists in employing in the electrolyte interposing between the anode and cathode an insoluble carbonate of a

metal whose sulfate when formed in the electrolyte is not detrimental, while screening the cathode from contact with said carbonate.

- 5 3. A process of electrolyzing a nickel sulfate solution with the use of a copper-nickel anode which consists in maintaining in contact with the anode a substantially insoluble re-agent capable of forming with copper an insoluble compound and a sulfate whose presence in the electrolyte is not detrimental, while screening the cathode from contact with such re-agent.
- 10

4. A process of electrolyzing a nickel sulfate solution with the use of a copper-nickel anode, which consists in interposing between the anode and cathode carbonate of calcium, while screening the cathode from contact with said carbonate.

Signed at Oakville, Ontario, this 4th day 15  
of August, 1917.

GEORGE A. GUESS.

Witnesses:

IRENE E. VANDIN,  
W. A. CHISHOLM.